

# UNITED STATES PATENT OFFICE.

AMZI L. BARBER, OF WASHINGTON, DISTRICT OF COLUMBIA.

## CONCRETE PAVEMENT.

SPECIFICATION forming part of Letters Patent No. 391,222, dated October 16, 1888.

Application filed July 18, 1888. Serial No. 280,323. (No specimens.)

*To all whom it may concern:*

Be it known that I, AMZI L. BARBER, a citizen of the United States of America, residing at Washington, in the District of Columbia, 5 have invented certain new and useful Improvements in Concrete Pavements, of which the following is a specification.

My invention relates to improvements in concrete pavements, and more particularly is 10 an improvement on the invention of E. J. De Smedt, patented December 20, 1887, No. 375,273.

The object of my invention is to thoroughly lock or cement the different layers or strata 15 of which the pavement is composed, so that there will be less liability to crack and disintegrate under the influence of the heat, cold, or moisture.

My invention consists, therefore, of a pavement having a base or foundation layer of 20 broken stone or gravel coated with a coal-tar paving-cement, upon which is placed a second and intermediate layer of smaller broken stone coated with coal-tar, upon which is placed the 25 wearing course or layer of asphaltum, heavy petroleum, or the residuum of petroleum, and fine sand.

In carrying out my invention the road-bed 30 is excavated to the proper depth, preferably about six inches below the surface of the pavement when completed, upon which is laid a foundation-layer of coarse broken stone or gravel about three inches in depth, (more or less,) said broken stone being coated with hot 35 coal-tar, preferably a cement of what is known to the trade as "No. 4 coal-tar distillate," in the proportion of about one gallon of the cement to each square yard of pavement. This base or foundation layer is well rolled and 40 rammed with a steam-roller, so that when compacted it will be about three inches in thickness, (more or less,) as above stated.

The second or binder course is composed of 45 clean broken stone or gravel, not exceeding one and one-fourth ( $1\frac{1}{4}$ ) inch in largest dimensions, the stone to be heated in any suitable manner and mixed with No. 4 coal-tar, distillate in the proportion of about one (1) gallon of the distillate to one (1) cubic foot of 50 stone. This binder-course is spread on the base or foundation course to form a layer of about one and one-half ( $1\frac{1}{2}$ ) inch in thickness when properly rolled or compacted. In

preparing the broken stone for this second or binder course care should be exercised to coat 55 each individual stone thoroughly, so that they will be cemented to the base-course and to each other when properly laid. This coating of the broken stone with the cement is best effected by the use of suitable mixing ma- 60 chinery.

The top or wearing surface or course is next placed upon the binder-course, and is to be about one and one-half inch in thickness when compacted. This top or wearing surface is 65 composed of refined Trinidad or other suitable natural asphaltum, heavy petroleum, or the residuum of petroleum, and fine sand.

The proportions of asphaltum and residuum of petroleum or heavy petroleum-oil used may 70 be varied within certain limits, but I prefer to use from fourteen to seventeen parts of residuum of petroleum to each one hundred parts of asphaltum, and sand sufficient to take up the bituminous compound and form a solid 75 mass when cold, and the sand and the asphaltic cement formed by the union of the asphalt and residuum are heated separately prior to being mixed.

The materials and combination of materials forming each layer or course of the pavement, except the first one of broken stone, are laid while in a heated condition, so that the second or binding course is joined or cemented to the base or bottom course and the top or 85 wearing course is cemented to the intermediate or binding course, and in this manner I produce a pavement which will be solid in all its parts and capable of withstanding the action of water and the expansions and contractions incident to thermal changes. 90

Having thus described my invention, what I claim is—

A concrete pavement consisting of a base or foundation layer of broken stone coated with 95 coal-tar or a coal-tar distillate, a binder or intermediate layer of smaller broken stone similarly coated, and a top or wearing course composed of asphaltum, residuum of petroleum, and sand, substantially as set forth. 100

In testimony whereof I affix my signature in presence of two witnesses.

AMZI L. BARBER.

Witnesses:

HENRY J. KEARNEY,  
JOHN P. WHITEHORN.